

## UNITED STATES PATENT OFFICE

2,082,814

PROCESS OF MAKING A SUBSTITUTE FOR  
WOOL FROM VISCOSE

Walther Zetsche and Hermann Faber, Premnitz,  
Germany, assignors to I. G. Farbenindustrie  
Aktiengesellschaft, Frankfort - on - the - Main,  
Germany

No Drawing. Application November 29, 1935,  
Serial No. 52,201. In Germany November 30,  
1934

5 Claims. (Cl. 18—54)

Our present invention relates to the manufacture of a substitute for wool from viscose.

One of its objects is a process of making an improved substitute for wool from viscose. Another object is a process of making well crimped staple fiber from viscose. Further objects will be seen from the detailed specification following hereafter.

According to the invention well crimped cellulose artificial fibers are obtained by cutting cellulose xanthate into staple threads and treating these with heated liquids to convert them into cellulose threads. It is preferable to stretch the xanthate threads in the coagulation bath or between the coagulation bath and the cutting machine. Any known device may be used for the stretching, for example rollers driven at different speeds, or rods set in staggered relationship in the path of the thread and thus cause the latter to change its direction. Also the stretching may be produced by use of a draft speed exceeding considerably the speed of expression of the xanthate. Spinning baths suitable for making the cellulose xanthate threads are ammonium sulfate solutions, with or without sodium sulfate. As decomposing liquids glycerin, glycol, sulfonated oil, such as sulfonated olive oil or castor oil are suitable. There may also be used aqueous solutions of high boiling point of inorganic salts, such as a calcium chloride solution, or a concentrated solution of sodium sulfate which has proved to be well adapted, aqueous solutions of organic acids, such as oxalic acid, alcohols of high boiling point, ethers of the hydroaromatic, aromatic and aliphatic series, ketones of high boiling point, such as cyclohexanone and their substitution products. The decomposition of the xanthate threads in a decomposing bath occupies a few seconds up to a few minutes in accordance with the temperature selected. The temperature may vary between about 60 and 150° C., and is preferably 120 to 130° C. It is also possible to decompose the threads at a temperature lower than 60°, however, the treatment lasts too long for practical purposes. After the decomposition the threads are separated from the decomposition liquid and freed by washing with water from the adhering chemicals, particularly the adhering decomposition liquid. From the washing liquid the substance used for decomposing the xanthate may be recovered by evaporation.

If glycerin, glycol, sulfonated oil, as well as organic liquids which dissolve sulfur are used for decomposing the xanthate fibers, the fibers

are at the same time desulfurized, so that separate desulfurizing is not necessary in this case.

The following is an example of the invention:

Viscose is spun from a nozzle having 800 perforations at 25° C. in a solution of ammonium sulfate of 30 per cent. strength; all the fiber bundles thus produced are united in a spinning machine to form thick bundles of several 1000 deniers. These bundles are now cut to staples and introduced into glycerin heated to 120° C. From the heated glycerin the crimped fibers are separated by means of conveyer sieves running over rollers or by any other known device. It is then freed, by washing with water, from the adhering glycerin and treated with solutions of scaping agents or brightening agents. The fibers thus made are dried and combed to produce a loose staple fiber sliver. The thread is thoroughly crimped, in which respect it approximates wool very closely.

Instead of the glycerin heated at 120° C. a concentrated solution of sodium sulfate boiling at about 103° C. may be used. The decomposition needs a little more time in view of the lower temperature.

What we claim is:

1. A process of making a substitute for wool which comprises squirting viscose into a precipitating bath capable of precipitating the viscose in the form of cellulose xanthogenate, assembling the spun threads to a thick fiber band, cutting the fiber band into staples, and converting the cellulose xanthogenate into cellulose hydrate by means of a liquid heated at 60 to 150° C.

2. A process of making a substitute for wool which comprises squirting viscose into a precipitating bath capable of precipitating the viscose in the form of cellulose xanthogenate, assembling the spun threads to a thick fiber band, cutting the fiber band into staples, and converting the cellulose xanthogenate into cellulose hydrate by means of a liquid heated at 120 to 130° C.

3. A process of making a substitute for wool which comprises squirting viscose into a precipitating bath capable of precipitating the viscose in the form of cellulose xanthogenate, assembling the spun threads to a thick fiber band, cutting the fiber band into staples, and converting the cellulose xanthogenate into cellulose hydrate by means of a liquid having a desulfurizing action heated at 60 to 150° C.

4. A process of making a substitute for wool which comprises squirting viscose into a precipitating bath capable of precipitating the viscose in the form of cellulose xanthogenate, assembling

the spun threads to a thick fiber band, cutting the fiber band into staples, and converting the cellulose xanthogenate into cellulose hydrate by means of glycerine heated at 120° C.

5. A process of making a substitute for wool which comprises squirting viscose into a precipitating bath capable of precipitating the vis-

cose in the form of cellulose xanthogenate, assembling the spun threads to a thick fiber band, cutting the fiber band into staples, and converting the cellulose xanthogenate into cellulose hydrate by means of a boiling salt solution.

WALTHER ZETZSCHE.  
HERMANN FABER.